

Feb. 23, 1965

R. J. FUERST

3,170,807

CONTACT COPY CORRECTING SHEET AND METHOD OF USING

Filed May 16, 1962

FIG. 1A



FIG. 1B



FIG. 2



FIG. 3



1, 1', 1'' = CARRIER SHEET  
2, 2', 10 = TRANSFER LAYER  
3, 3', 12 = TAKE-UP LAYER  
6 = TYPEWRITER ROLLER  
7, 8 = TYPEWRITER KEYS



FIG. 4

BY

INVENTOR  
Robert J. Fuerst  
By:  
Michael J. Stricker  
Attn:

# United States Patent Office

3,170,807

Patented Feb. 23, 1965

1

3,170,807

## CONTACT COPY CORRECTING SHEET AND METHOD OF USING

Robert J. Fuerst, White Plains, N.Y., assignor to Kores  
Manufacturing Corporation, New York, N.Y.

Filed May 16, 1962, Ser. No. 195,289

3 Claims. (Cl. 117—2)

The present invention relates to a contact copy correcting sheet and method and, more particularly, the present invention is concerned with a correcting sheet and with a method of correcting contact copies which may be used in connection with the copy paper or the like which is disclosed in the U.S. application, Serial No. 136,711, by Eugen Strauss, entitled: "Copy Paper or the Like," now abandoned.

Certain difficulties are encountered in correcting of copies made with carbonless copy paper such as the copy paper described in application, Serial No. 136,711. Carbonless copy paper may be used, for instance, in the form of a sheet assembly composed of a plurality of sheets, one of which is provided on one face with a transfer layer which is adapted to be placed in face-to-face contact with another sheet carrying on its contacting face a take-up layer, the transfer layer consisting essentially of a resinous substance selected from the group consisting of polyvinyl acetate, mixed polymerizes of polyvinyl acetate, colophonium, polymethylacrylate, polymethylmethacrylate, polycarbonates, polystyrene, polychloroprene, styrene-butadiene copolymers, cumarone resins, and cumarone-phenol resins in an amount of about 4-20% by weight of the transfer layer, of at least one plasticizer for the resinous substance, of at least one organic fixing agent selected from the group consisting of tannic acid, gallic acid, digallic acid, salicylic acid, phenyl salicylate, 4 - butyl-phenyl-salicylate, 5-chloro-2-hydroxy-benzophenone, 2,4-dibenzoyl-resorcin phenol and pyrogallic acid, of at least one inorganic substance of substantially colloidal particle size and selected from the group consisting of bentonite, kaolin, calcium carbonate, calcium sulfate, calcium phosphate and zinc oxide, and of a pigment; and the take-up layer consisting essentially of a dry resinous substance selected from the group consisting of acrylic polymers, vinyl polymers, acrylic-vinyl mixed polymers, polydolefines, dolefine-styrene mixed polymers, polycarbonates, colophonium, copal, abietic-maleic resin and cumarone resins and of at least one plasticizer in which the resinous substance is soluble, preferably in an amount of 10-50% by weight of the weight of the resinous substance. The composition of the various layers is described in more detail in the above-mentioned U.S. patent application, Serial No. 136,711.

The difficulties encountered in the use of this assembly include that the resulting copy cannot be removed neatly with an ordinary eraser. Furthermore, the coating of the reverse side of the original, i.e., the transfer, layer is removed completely at those portions where pressure is applied and the corresponding portion of the transfer layer is adhered to the take-up layer of the underlying sheet, and therefore no reproducing medium is left at such depleted portion of the transfer layer for use upon subsequent and repeated exertion of pressure to form a corrected copy on the take-up layer.

It is therefore an object of the present invention to provide a correcting sheet and method for correcting copies produced, for instance, with such sheet assemblies as described above, in such a manner that the incorrect copy, for instance a typographical error, can be removed and a correct copy can be produced in place of the removed incorrect copy.

It is a further object of the present invention to achieve

2

the above described objects in a simple and economical manner.

Other objects and advantages of the present invention will become apparent from a further reading of the description and of the appended claims.

With the above and other objects in view, the present invention contemplates for use in an assembly for correcting contact copy of the type formed by placing one sheet which is provided on one face with a transfer layer having a first color in face to face contact with another sheet which is provided with a take-up layer having a second color contrasting with the first color, with the transfer and take-up layers contacting each other, and applying pressure to spaced portions of the other face of the one sheet so that corresponding portions of the transfer layer thereof will be transferred onto the take-up layer of the other sheet, in combination, a correcting sheet comprising a carrier sheet provided on one face thereof with a first layer of substantially the first color adapted upon application of pressure to adhere to the transfer layer of the first sheet, and also adapted to be subsequently transferred by application of pressure from the first sheet to the take-up layer of another sheet, and provided on its other face with a second layer of substantially the second color and adapted upon application of pressure to adhere to the take-up layer of the second sheet forming part thereof, whereby upon interposition of the correcting sheet between the one and the other sheet with the first layer of the correcting sheet contacting the transfer layer of the first sheet and the second layer of the correcting sheet contacting the take-up layer of the second sheet and application of pressure to the spaced portions of the thus formed sheet assembly the portions of the faces of the first and second sheet to which the spaced pressure is applied will be covered by corresponding portions of the respective layers of the correcting sheet.

The present invention is also concerned with an assembly for correcting contact copy of the type formed by placing one sheet which is provided on one face with a transfer layer in face to face contact with another sheet which is provided with a take-up layer, and the transfer and take-up layers contacting each other, and applying pressure to spaced portions of the other face of the one sheet so that corresponding portions of the transfer layer thereof will be transferred onto the take-up layer of the other sheet, in combination, a first sheet provided on one face with the transfer layer, a second sheet provided on one face with a take-up layer, the first and second sheets being superposed with the transfer and take-up layers adjacent to each other, and a correcting sheet interposed between the superposed first and second sheets, the correcting sheet comprising a carrier sheet provided on one face thereof with a first layer adapted upon application of pressure to adhere to the transfer layer of the first sheet, and provided on its other face with a second layer adapted upon application of pressure to adhere to the take-up layer of the second sheet, the one face of the interposed correcting sheet being adjacent to the transfer layer of the first sheet and the other face of the correcting sheet being adjacent to the take-up layer of the second sheet.

The present invention further comprises in a method of correcting contact copy of the type formed by placing one sheet which is provided on one face with a transfer layer in face to face contact with another sheet which is provided with a take-up layer, with the transfer and take-up layer contacting each other, and applying pressure to spaced portions of the other face of the one sheet so that corresponding portions of the transfer layer thereof will be transferred onto the take-up layer of the other sheet forming copy thereon, the steps of interposing between superposed transfer and take-up layers having the copy formed on the take-up layer a correcting sheet carrying on

one face a transfer layer and on the other face a take-up layer, with the take-up layer of the correcting sheet facing the copy formed on the take-up layer of the other sheet and the transfer layer of the correcting sheet facing the transfer layer of the one sheet, and applying spaced pressure corresponding to the configuration of the copy to the first and second sheet with the correcting sheet interposed therebetween so that portions of the transfer and take-up layers of the correcting sheet corresponding to the copy will be transferred to corresponding portions of the transfer and take-up layers-carrying faces of the one and of the other sheet, respectively, thereby obliterating the previously formed copy thereon and restoring the transfer and take-up layers of the one and of the other sheet to their previous condition.

The novel features which are considered as characteristic for the invention are set forth in particular in the appended claims. The invention itself, however, both as to its construction and its method of operation, together with additional objects and advantages thereof, will be best understood from the following description of specific embodiments when read in connection with the accompanying drawings, in which:

FIG. 1 (comprising FIGS. 1a and 1b) is a diagrammatic, cross sectional illustration of the transfer of copy, 25 using copy sheets of the type mentioned above, which copy may be corrected in accordance with the present invention as illustrated in the following figures of the drawing.

FIG. 2 illustrates a portion of what is shown in FIG. 1b, namely, the copy sheet 1, 2 and the copy sheet 3, 1', 2' in the condition in which these sheets are shown in FIG. 1b, i.e., after copy has been transferred from sheet 1, 2 to intermediate copy sheets 3, 1', 2';

FIG. 3 illustrates the interposition of a correcting sheet 35 according to the present invention between the two sheets shown in FIG. 2, and

FIG. 4 illustrates how repeated application of the pressure which formed the copy as shown in FIG. 2, however, with the correcting sheet interposed between the two sheets of FIG. 2 will correct, i.e., obliterate the copy which had been formed according to FIGS. 1 and 2.

Referring now to the drawings, and particularly to FIG. 1, the same illustrates the making of copies with three copy sheets. Copy sheet 1, 2 comprises a carrier sheet 1 and a transfer layer 2. It is placed adjacent a copy sheet 1', 2', 3, which comprises a carrier sheet 1', having on one face thereof a take-up layer 3, and on the other face thereof a transfer layer 2'. Sheet 3, 1', 2' is placed between sheet 1, 2 and a further copy sheet 1'', 3'' comprising a carrier sheet 1'' and a take-up layer 3''. This assembly of three sheets is placed against the typewriter roller 6 and when the typewriter keys 7 and 8 strikes the sheet, the corresponding portion of the transfer layer 2 will be adhered to take-up layer 3 of intermediate copy sheet 3, 1', 2' and the corresponding portion of transfer layer 2' from intermediate copy sheet 3, 1', 2' to carrier sheet 1'', 3'', where it adheres to take-up layer 3''.

For illustrating the present invention it will suffice to show in FIGS. 2, 3 and 4 only two copy sheets, namely sheet 1, 2; and the adjacent sheet 3, 1', 2'.

According to FIG. 3, a correcting sheet 10, 11, 12, is interposed between the two sheets of FIG. 2.

Correcting sheets 10, 11, 12 comprises a carrier sheet 11, having a transfer layer 10, facing the remaining portions of transfer layer 2 which adheres to carrier sheet 1, and carrier sheet 11 carries at its opposite face a take-up layer 12 which faces take-up layer 3 of the sheet comprising take-up layer 3, carrier sheet 1' and transfer layer 2', whereby it must be noted that now portions of transfer layer 2 forming the copy on sheet 1' adhere to take-up layer 3.

Upon striking the first sheet in the same manner as described in connection with FIG. 1b, the portions of transfer layer 10 of the correcting sheet which are thus

exposed to pressure will separate from the correcting sheet and will be adhered to carrier sheet 1 so as to fill the voids in transfer layer 2 which were formed upon initial exertion of pressure in accordance with FIG. 1b. Simultaneously, portions of take-up layer 12 which are exposed to pressure will separate from carrier sheet 11, of the correcting sheet and will be superposed upon the portions 2 of the initial transfer layer 2 which upon originally exerting pressure were adhered to take-up layer 3 of carrier sheet 1'.

In this manner transfer layer 2 on carrier sheet 1 is restored and will consist now of the residual portions of the original transfer layer 2 and the fill-in provided by portions of transfer layer 11, while the copy formed on take-up layer 3 of carrier sheet 1' and which consisted of the portions of transfer layer 2 which upon initial exertion of pressure had separated from carrier sheet 1, will be made invisible by superposition of portions of take-up layer 12, preferably having a color similar to the color of take-up layer 3.

Upon subsequent removal of the correcting sheet 11 with the portions of layers 10 and 12 which were not subjected to pressure still adhering thereto, the carrier sheet 1, with transfer layer 2-10 thereon and the carrier sheet 1' with take-up layer 3-12 thereon, are freed of any previously produced copy, and the sheets which are still in the typewriter may be imprinted again by operation of the typewriter keys.

While, as illustrated, only the interposition of one correction sheet between two carrier sheets 1 and 1' with the respective layers thereon has been shown and described, it is of course possible to interpose a plurality of correction sheets between a correspondingly greater number of carrier sheets which, in the illustrated sequence, carry on one face a transfer layer and on the other face a take-up layer. The bottom sheet need not carry a transfer layer at its face contacting the roller of the typewriter, and the top sheet need not carry a take-up layer at its face which will come in direct contact with the typewriter keys.

Thus, according to the present invention the correcting sheet comprises a carrier sheet of paper or other suitable medium which is coated on one side with a surface layer having substantially the same color as the take-up layer of the copy sheets, generally a white layer, and on its other side with a transfer layer which preferably will be dark grey or black, again corresponding to the color of the transfer layer of the copy sheets.

Again assuming that copy was produced in a typewriter and that a typographical error has been made, such error is corrected in the following manner: the correcting sheet is inserted between the original and the first copy sheet or, if there are more copies than the original and the first copy, other correcting sheets are inserted between the first and second copy sheet, and so forth, whereby each correcting sheet is inserted in such a manner that its white surface, i.e., its take-up layer faces the take-up layer of the respective copy sheet. In other words, the white or take-up layer of the correcting sheet 60 faces away from the typewriter keys, while the grey or black, transfer layer of the correcting sheet faces towards the typewriter keys, and thus towards the transfer layer of the adjacent copy sheet. The typographical error is now repeated at the identical location. As a result, the white surface of the correcting sheet releases a white pigment which will cover or obliterate the error appearing on the copy in grey or black or whatever other contrasting copy is used for the transfer layer, while at the same time portions of the grey or black or otherwise contrastingly colored transfer layer on the correcting sheet will be released therefrom and will cover the portion of the adjacent carrier sheet of the copy sheet from which the transfer layer previously had been removed by initially producing the typographical error.

Thereafter, the correcting sheet is removed from be-

tween any two adjacent copy sheets and between the original and the first copy sheet, and it is apparent that the transfer and take-up layers of the original and copy sheets have now been restored to the condition in which they were prior to typing the typographical error. In this manner it is now possible to type correctly at the place where previously the typographical error occurred. The coating of the original now having been replaced reproduces or transfers the corrected typing onto the take-up layer of the copy sheet over the error which is now covered with the white coating originating from the take-up layer of the correcting sheet.

It is of course possible to erase in conventional manner original image produced on the top sheet by direct pressure contact with the typewriter ribbon.

The correcting sheet according to the present invention thus will consist essentially of a carrier sheet having on one face a preferably white layer which will be capable of covering the previously formed image on the copy sheet and having on its opposite face a layer which is adapted to restore the transfer layer of the original sheet or of a copy sheet by transferring transfer layer material to those portions of the carrier sheet of the original or copy sheet from which transfer layer had been removed by the previous typing action.

The take-up layer of the correcting sheet which generally will be of white color will consist of suitable pigments, binders and softeners. Minor variations of the proportions of binder and softener relative to each other will produce very considerable variations in the hiding power or covering effect which transferred portions of the take-up layer will have relative to the underlying imprint.

The following examples of correcting sheets according to the present invention are given as illustrative only, without, however limiting the invention to the specific details of these examples.

By using as carrier sheet of the correcting sheet a strongly calendered and glued paper, or a paper of the artificial parchment type, i.e., a paper which has very little absorptive capacity, it is possible to produce clear and sharp edged corrections with a relatively small percentage amount of softeners such as butyl Cellosolve, Palatinol, Myverol or Cereclor. Pergamyn is a grease-proof imitation parchment paper made from sulfate pulp; Myverol is a glyceride derived from lard; Cereclor is a chloroparaffin containing 42% of chlorine, Cellosolve broadly is 2-ethoxy-ethanol; the Palatinol softeners are phthalic acid derivatives well known in the art.

When the carrier sheet and the correcting sheet consist of only slightly calendered and slightly glued paper, then the percentage of softeners must be increased.

The usually black or dark grey transfer layer of the correcting sheet which will serve to regenerate the transfer layer of the copy sheets and thus to permit again to produce copy from portions thereof which previously had been subjected to pressure, may be chosen from various groups of materials.

However, in this connection it is important, that the adherence of the transfer layer of the correcting sheets to the carrier sheet must be somewhere in-between the degree of adherence of the transfer layer and of the take-up layer of the copy sheets which are to be regenerated.

It is therefore desirable, to adjust the specific composition of the transfer layer as well as of the take-up layer of the correcting sheets to the type of paper or the like which forms the carrier sheet of the correcting sheet.

#### Example I

The correcting sheet comprises a carrier sheet of smooth calendered or artificial parchment paper weighing between 35 and 40 gr./m.<sup>2</sup>.

The white or take-up layer is produced by mixing:

37.50 parts by weight titanium dioxide

13.50 parts by weight lithopone (80% zinc sulfide)

2.10 parts by weight Cereclor 42 (chloroparaffin 42% chlorine)

1.05 parts by weight Myverol 18-07 (glyceride of hydrated lard)

0.80 part by weight Palatinol AH (dioctylphthalate)

20.80 parts by weight ethanol 94%

0.04 part by weight Mark II A (a colloidal carbon for use in inks, produced by Columbian Carbon Company, N.Y.)

10 The thus formed mixture is ground for one hour in a ball mill and thereafter the following solution is admixed under stirring:

3.80 parts by weight pulverulent ethylcellulose N 100 (a cellulosic ether 47.5-49% ethoxyl; 80-105 cps. viscosity at 5% concentration in 80% ethanol and 20% toluene by weight at 25° C.)

3.30 parts by weight butyl Cellosolve stearate

1.40 parts by weight Lucite 44 (an acrylic resin m-butyl methacrylate polymer, produced by Du Pont)

29.93 parts by weight trichloroethylene

The amount of the thus formed mixture which is applied to the carrier sheet depends on the quality of the carrier sheet. Generally, the smoother the carrier sheet

25 the less of the mixture will be applied. Using as carrier sheet a paper of the type described above, the mixture preferably will be applied to one face thereof so as to form thereon a layer weighing between about 35 and 40 gr./m.<sup>2</sup>.

30 The dark, or transfer, layer is formed of a mixture of 50 parts by weight Armeen HT (octodecylamine)

20 parts by weight Black Toner (a carbon black "Toner" produced by Columbian Carbon Co., N.Y.)

10 parts by weight English kaolin

25 parts by weight tricresyl phosphate

The above mixture is heated so as to be in flowable state and applied to the other face of the carrier sheet to form thereon a layer weighing 10 gr./m.<sup>2</sup>.

#### Example II

The carrier sheet and take-up layer are similar to those described in Example I. The transfer or dark layer consists of:

45 22.5 parts by weight crude montan wax

21.5 parts by weight petroleum jelly

24 parts by weight mineral oil II (Engler viscosity 2° at 50° C.)

27 parts by weight Furnex (semi-reinforcing furnace-carbon-black)

5 parts by weight kaolin

10 parts by weight Abitol (hydroabietil alcohol—Hercules Powder)

55 This mixture is applied so as to form a layer on one face of the carrier sheet weighing between 12 and 22 gr./m.<sup>2</sup>.

The above formula can be improved by the incorporation of about 32.5% instead of 22.5% of crude montan wax, whereby the pressure-transferred indicia will appear more clearly and sharply defined and the layer will be more resistant against smearing.

#### Example III

65 The correcting sheet comprises a carrier sheet of Perkallin (a filled or partially transparent artificial parchment paper such as onionskin paper) paper weighing 40 gr./m.<sup>2</sup>.

The white or take-up layer is produced by mixing:

70 37.50 parts by weight titanium dioxide

13.50 parts by weight lithopone (80% zinc sulfide)

2.10 parts by weight Cereclor 42 (chloroparaffin 42% chlorine)

1.05 parts by weight Myverol 18-07 (glyceride of hydrated lard)

0.80 part by weight Palatinol AH (dioctylphthalate)  
20.80 parts by weight ethanol 94%

The thus formed mixture is finely ground and thereafter mixed under stirring with a solution consisting of:

3.50 parts by weight solution of 10% ethylcellulose N 100 in 90% ethanol  
3.20 parts by weight butyl Cellosolve stearate  
1.20 parts by weight Lucite 44 (Du Pont—acryl)  
25.00 parts by weight trichloroethylene  
10.25 parts by weight Mark II A

The thus formed mixture is applied to the carrier sheet so as to form on one face thereof a layer weighing 25 gr./m.<sup>2</sup>.

The dark transfer layer is formed by mixing:

50 parts by weight Armeen HT  
20 parts by weight Black Toner  
5 parts by weight Palatinol C (dibutylphthalate)  
10 parts by weight castor oil  
10 parts by weight English kaolin

The thus formed mixture is applied to the other face of the carrier sheet so as to form thereon a layer weighing between 5 and 7 gr./m.<sup>2</sup>.

#### Example IV

The carrier sheet and the take-up layer are the same as described in Example I.

The dark transfer layer is formed by mixing two solutions, namely a solution "A" which is formed of:

20 parts by weight Crilat D 131 (a 50% aqueous emulsion of methacrylate produced by Montecatini)  
20 parts by weight Palatinol C (dibutylphthalate BASF)  
500 parts by weight ethanol 94%  
5 parts by weight ammonium hydroxide 28 Be

Solution "B" consists of:

400 parts by weight ethanol 94%, and  
850 parts by weight of a paste "C" having the following 40 composition

Paste "C" is an intimate mixture of:

2.50 parts by weight carbon black (Peerless Mark II A)  
14.00 parts by weight methylglycol (methyl Cellosolve)  
39.00 parts by weight titanium dioxide (titanium white)  
18.00 parts by weight kaolin  
13.00 parts by weight Palatinol C (dibutylphthalate)  
13.50 parts by weight castor oil

Paste "C" is produced by passing the above mixture 3 times through a three-roller refiner.

Solutions "A" and "B" are now intimately mixed under stirring so as to become homogenized and the thus formed mass is applied to one face to the, for instance, smooth calendered paper carrier sheet so as to form thereon a layer weighing between about 39 and 40 gr./m.<sup>2</sup>.

It will be understood that each of the elements described above, or two or more together, may also find a useful application in other types of copy correcting sheets differing from the types described above.

While the invention has been illustrated and described as embodied in a correcting sheet for copies produced without the interposition of carbon papers, it is not intended to be limited to the details shown, since various modifications and structural changes may be made without departing in any way from the spirit of the present invention.

Without further analysis, the foregoing will so fully reveal the gist of the present invention that others can by applying current knowledge readily adapt it for various applications without omitting features that, from the standpoint of prior art, fairly constitute essential characteristics of the generic or specific aspects of this invention and, therefore, such adaptations should and are intended

to be comprehended within the meaning and range of equivalence of the following claims.

What is claimed as new and desired to be secured by Letters Patent is:

- 5 1. An assembly for correcting contact copy of the type formed by placing one sheet which is provided on one face with a transfer layer in face to face contact with another sheet which is provided with a take-up layer, with said transfer and take-up layers contacting each other, and applying pressure to spaced portions of the other face of said one sheet so that corresponding portions of said transfer layer thereof will be transferred onto the take-up layer of said other sheet, in combination, a first sheet provided on one face with a transfer layer; a second sheet provided on one face with a take-up layer, said first and second sheets being superposed with said transfer and take-up layers adjacent to each other; and a correcting sheet interposed between said superposed first and second sheets, said correcting sheet comprising a carrier sheet provided on one face thereof with a first layer which when superposed upon said transfer layer of said one sheet will upon application of pressure become detached from its carrier sheet and adhere to said one sheet, and provided on its other face with a second layer which 20 when superposed upon said take-up layer of said other sheet will upon application of pressure become detached from its carrier sheet and adhere to said take-up layer of said other sheet, said one face of said interposed correcting sheet being adjacent to said transfer layer of said one sheet and said other face of said correcting sheet being adjacent to said take-up layer of said other sheet.
- 15 2. In a method of correcting contact copy of the type formed by placing one sheet which is provided on one face with a transfer layer in face to face contact with another sheet which is provided with a take-up layer, with said transfer and take-up layers contacting each other, and applying pressure to spaced portions of the other face of said one sheet so that corresponding portions of said transfer layer thereof will be transferred onto the take-up layer of said other sheet forming copy thereon, the steps of interposing between superposed transfer and take-up layers having said copy formed on said take-up layer a correcting sheet carrying on one face a transfer layer which when superposed upon said face of said one sheet provided with a transfer layer will 30 upon application of pressure become detached from said correcting sheet and adhere to said one sheet, and carrying on the other face a take-up layer, which when superposed upon said take-up layer of said other sheet will 35 upon application of pressure become detached from said correcting sheet and adhere to the take-up layer of said other sheet with said take-up layer of said correcting sheet facing said copy formed on said take-up layer of said other sheet and said transfer layer of said correcting sheet facing said transfer layer of said one sheet; and applying spaced pressure corresponding to the configuration of said copy to said first and second sheet with said 40 correcting sheet interposed therebetween so that portions of said transfer and take-up layers of said correcting sheet corresponding to said copy will be transferred to corresponding portions of said transfer and take-up layers carrying faces of said one and of said other sheet, respectively, thereby obliterating said previously formed copy thereon and restoring said transfer and take-up layers of said one and of said other sheet to their previous condition.
- 45 3. A correcting sheet adapted for use in an assembly for correcting contact copy of the type formed by placing one sheet which is provided on one face with a transfer layer in face to face contact with another sheet which is provided with a take-up layer, with said transfer and take-up layers contacting each other, and by applying pressure to spaced portions of the other face of said one sheet so that corresponding portions of said transfer layer thereof will be transferred onto the take-up layer of said 50 sheet.
- 55 4. A method of correcting contact copy of the type formed by placing one sheet which is provided on one face with a transfer layer in face to face contact with another sheet which is provided with a take-up layer, with said transfer and take-up layers contacting each other, and by applying pressure to spaced portions of the other face of said one sheet so that corresponding portions of said transfer layer thereof will be transferred onto the take-up layer of said sheet.
- 60 5. An assembly for correcting contact copy of the type formed by placing one sheet which is provided on one face with a transfer layer in face to face contact with another sheet which is provided with a take-up layer, with said transfer and take-up layers contacting each other, and applying pressure to spaced portions of the other face of said one sheet so that corresponding portions of said transfer layer thereof will be transferred onto the take-up layer of said sheet.
- 65 6. A method of correcting contact copy of the type formed by placing one sheet which is provided on one face with a transfer layer in face to face contact with another sheet which is provided with a take-up layer, with said transfer and take-up layers contacting each other, and by applying pressure to spaced portions of the other face of said one sheet so that corresponding portions of said transfer layer thereof will be transferred onto the take-up layer of said sheet.
- 70 7. An assembly for correcting contact copy of the type formed by placing one sheet which is provided on one face with a transfer layer in face to face contact with another sheet which is provided with a take-up layer, with said transfer and take-up layers contacting each other, and applying pressure to spaced portions of the other face of said one sheet so that corresponding portions of said transfer layer thereof will be transferred onto the take-up layer of said sheet.
- 75 8. A method of correcting contact copy of the type formed by placing one sheet which is provided on one face with a transfer layer in face to face contact with another sheet which is provided with a take-up layer, with said transfer and take-up layers contacting each other, and by applying pressure to spaced portions of the other face of said one sheet so that corresponding portions of said transfer layer thereof will be transferred onto the take-up layer of said sheet.

other sheet, said correcting sheet comprising, in combination, a carrier sheet provided on one face thereof with a coating of a detachable dark colored transfer material which when superposed upon said transfer layer of said one sheet will upon application of pressure become detached from said carrier sheet and will adhere to said one sheet and restore said transfer layer thereof, and provided on its other face with a coating of a detachable light colored take-up material which when superposed upon said take-up layer of said other sheet will upon application of pressure become detached from said carrier sheet and adhere to said other sheet and restore said take-up layer thereof, whereby upon interposition of said correcting sheet between said one and said other sheet with said coating of detachable dark colored transfer material of said correcting sheet contacting said transfer layer of said one sheet and said coating of detachable light colored take-up material of said correcting sheet

10

5

contacting said take-up layer of said other sheet and application of pressure to said portions of the thus formed sheet assembly, the portions of said faces of said one and said other sheet which are directed towards each other and to which said pressure is applied will be covered by corresponding portions of said respective coatings of said correcting sheet.

## References Cited in the file of this patent

## UNITED STATES PATENTS

|           |         |               |
|-----------|---------|---------------|
| 701,443   | Wilson  | June 3, 1902  |
| 1,845,568 | Strawn  | Feb. 16, 1932 |
| 2,168,098 | Groak   | Aug. 1, 1939  |
| 3,096,867 | Kuhlman | July 9, 1963  |

## FOREIGN PATENTS

|         |               |              |
|---------|---------------|--------------|
| 528,589 | Great Britain | Nov. 1, 1940 |
|---------|---------------|--------------|